

Patented July 17, 1928.

1,677,674

# UNITED STATES PATENT OFFICE.

LESLIE E. HOWARD AND ALLEN D. POTTS, OF LOCKPORT, NEW YORK, ASSIGNEES TO SIMONDS SAW AND STEEL COMPANY, OF FITCHBURG, MASSACHUSETTS, A CORPORATION OF MASSACHUSETTS.

## ART OF PRODUCING PERMANENT MAGNETS.

No. Drawing. Application filed October 9, 1926. Serial No. 140,671.

This invention relates to permanent magnets and to a method for making the same.

In the art of making magnets, it has long been a matter of common knowledge that 5 carbon steels which have been heated and then quenched thereby acquire the property of retaining a considerable proportion of any magnetic flux or magnetization which may be subsequently induced in them by the application of exterior forces.

Certain of the alloy steels, such as tungsten-, chrome-, chrome-tungsten-steels, and the like, also manifest per se, this property of retaining an impressed magnetic flux, 15 more permanently and in a greater proportion than do the straight carbon steels.

In the commercial production of magnets, however, it is usually necessary that they conform to certain shapes and sizes in order 20 to adequately serve the several purposes for which they may be intended. This requires either that the metal be heated and shaped while hot (as by forming under a drop hammer or the like) or that the metal be given 25 a preliminary annealing or reheating treatment and then shaped, when cold stamping or bending operations are to be carried out.

Such heating and cooling or annealing of either carbon or alloy steels (and especially 30 of tungsten alloy steels) tends to greatly reduce the degree or proportional amount of residual magnetization which the metal is capable of acquiring or retaining under demagnetizing influences.

35 For example, if the metal is shaped without any heating whatever and, after forming, is heated to the proper temperature and hardened by quenching, it will always be superior in its magnetic qualities and properties to one which has been, for instance, annealed or heated in the forming operation and allowed to cool more or less slowly. In other words, subsequent hardening of the 40 steel is inadequate to overcome the effects of previous heat treatments, such as annealing, or to restore the capacity or magnetic quality of the alloy for acquiring a permanent magnetization. This deterioration of magnetic quality by heat is more apparent with 45 the alloy steels than with straight carbon steels, and is especially marked with the tungsten-steels which are otherwise characterized by manifesting a particularly high capacity for retaining residual magnetism.

Accordingly it is an object of the present 55 invention to provide a magnet steel which may be shaped, annealed, bent, and otherwise treated, as may be required, without losing its capacity or quality for becoming and remaining substantially permanently 60 magnetized to a high proportionate degree by any magnetic flux subsequently impressed thereon or induced therein, and a method for making permanent magnets therefrom. Other objects of the invention will appear 65 from the preceding and following disclosure, and from the claims.

The present invention includes the discovery 70 that the addition or presence of vanadium in steel renders the resulting compound or alloy not only susceptible of initially retaining a high degree of residual magnetization (proportionate, for example, to the impressed magnetic flux to which it may be subjected), but also capable of retaining such magnetic quality in spite of annealing or other heat treatment and the effects of mechanical working and manipulation of the metal before final hardening. A still further discovery, forming a part of 75 the present invention, is that such improvement of the qualities of magnetization and permanency are manifested to a greater degree with the magnetic alloy steels and more particularly with those alloy steels 80 which are subject to the inhibitions above noted, namely, steels containing tungsten.

The invention will accordingly be described with reference to its application to tungsten alloy steels, but it is to be understood that such description is illustrative of 90 its adaptations in actual practice and not by way of limitation of the invention.

The procedure of the invention comprises 95 generally the incorporation of vanadium with steel or an alloy steel in appropriate or sufficient quantity, and preferably in a state of relatively uniform dissemination throughout the total metallic mass, as by direct addition to the molten metal. The 100 resulting alloy may then be shaped and treated in substantially any manner required including slow temperature changes and mechanical operations. This shaped metal is then hardened (as by heating and quenching) and finally magnetized in the 105 usual way.

Such additions of vanadium to steel result

in producing a more stable condition of the resulting metal or alloy, with corresponding freedom from the troubles and difficulties incident to or resulting from the annealing, 5 heating and forming operations which have been alluded to above. A proportion of .15% to 1.00% of vanadium constitutes a preferred range for magnets having such shapes as to require usual heat treatment 10 for shaping purposes.

This preservation of the magnetic quality of the steel permits of permanent magnets being successfully fashioned while hot or annealed to facilitate punching, drilling, 15 tapping of holes and other like operations in the cold without lowering their capacity for subsequent acquisition of permanent magnetism.

While the invention has been more particularly described with reference to its adaptation to tungsten steel, it is to be understood that like results may be attained with carbon steels and other alloy steels such as chrome steel, chrome-tungsten steel 25 and the like. Other modifications and adaptations of the invention may and ordi-

narily will be resorted to in the practical application of the same for commercial operations and uses, but such modifications and adaptations are to be considered as comprehended by the above disclosure and included within the terms of the following claims.

We claim:

1. An alloy steel containing vanadium in 35 quantity sufficient to permit the steel to be reheated and shaped without destroying its magnetic quality and characterized by a substantially permanent magnetization.

2. A permanent magnet comprising steel 40 having a vanadium content of .05 to 1.00%, reheated and shaped to the desired form, hardened and magnetized.

3. A permanent magnet comprising a tungsten steel having a vanadium content 45 of .05 to 1.00%, and characterized by a substantially permanent magnetization.

Signed by us at Lockport, New York, this 5th day of October, 1926.

LESLIE E. HOWARD.  
ALLEN D. POTTS.